

# UNITED STATES PATENT OFFICE.

RUDOLF LINKMEYER, OF HERFORD, GERMANY.

## MANUFACTURE OF ARTIFICIAL THREADS FROM SOLUTIONS OF CELLULOSE.

No. 795,526.

Specification of Letters Patent.

Patented July 25, 1905.

Application filed April 4, 1905. Serial No. 253,858.

*To all whom it may concern:*

Be it known that I, RUDOLF LINKMEYER, textile engineer, a subject of the Emperor of Germany, residing at Herford, in the Empire of Germany, have invented certain new and useful Improvements in the Manufacture of Artificial Threads from Solutions of Cellulose, of which the following is a specification.

It is known that artificial threads presenting the luster of silk may be produced by effecting the solution of cellulose in ammoniacal oxid of copper and in then precipitating the cellulose from its solution. Cellulose cannot, however, be readily dissolved directly in large quantities in ammoniacal oxid of copper in such a manner that the solution may present a degree of concentration sufficient to permit of the precipitation. Solution may in certain cases require eight days. Numerous processes have already been suggested for facilitating the solution, the greater number of these processes being based upon the energetic action of fixed alkalies before the solution with a view to producing a previous dehydration of the cellulose. All these processes present serious defects. In particular they are complicated by the fact that the previous treatment and the solution of the cellulose must be effected with different chemical agents.

The process which forms the subject of the present invention obviates these defects, the preliminary treatment and dissolving the cellulose being effected with the same reagents employed in solutions only the degree of concentration of which differs.

This process consists, broadly, in first of all producing in a first weak bath of ammoniacal oxid of copper a swelling of the fibers and a deposit of oxid of copper upon them and in then effecting solution in a concentrated solution of ammoniacal oxid of copper. In this manner a solution is obtained the very pronounced viscosity of which is extremely advantageous for spinning.

It has been found that the solution of the cellulose is effected very efficiently if the cotton, bleached or boiled for some hours, is first of all placed, either in a dry or humid condition, in a weak bath of ammoniacal oxid of copper, to which may be added with advantage a small quantity of caustic soda. This first bath serves to soften, swell, and dis-aggregate to some extent the fibers and to

fix upon them the oxid of copper dissolved by the ammonia. The fibers then dissolve speedily and readily in a concentrated solution of ammoniacal oxid of copper. By proceeding in this manner the conversion of the cellulose into oxycellulose or the hydration of the fibers is avoided. Further, the success of the solution depends less upon the temperature than upon the other processes. Solution takes place equally well at 10° to 15° centigrade as at a lower temperature.

The process may be applied as follows: About seven grams of cotton freed from grease or bleached are placed in, say, one hundred and fifty to one hundred and eighty cubic centimeters of ammoniacal oxid of copper containing about twelve grams of copper and ninety grams of ammonia per liter and to which there has previously been added, say, six cubic centimeters of caustic soda at 40° to 50° Baumé. After remaining for two to three hours or longer in this bath the fibrous material is removed and freed by pressure from the liquid in excess, and it is then dissolved in one hundred grams of ammoniacal oxid of copper containing, say, sixteen to eighteen grams of copper and two hundred grams of ammonia per liter. In this manner a thick solution is speedily obtained which may be diluted with water. After careful filtration this solution is ready for conversion into threads of artificial silk by an appropriate treatment.

What I claim, and desire to secure by Letters Patent of the United States, is—

1. A process for the solution of cellulose in ammoniacal oxid of copper, consisting in placing the cellulose first of all in a weak solution of ammoniacal oxid of copper and then in a concentrated solution of ammoniacal oxid of copper.

2. A process for the solution of cellulose in ammoniacal oxid of copper, consisting in placing the cellulose first of all in a weak ammoniacal-oxid-of-copper solution, in the presence of caustic soda, and then in a concentrated solution of ammoniacal oxid of copper.

In testimony whereof I have hereunto set my hand, in presence of two subscribing witnesses, this 21st day of March, 1905.

RUDOLF LINKMEYER.

Witnesses:

W. W. TIEKVATRIM,  
T. V. KIRKPATRICK.